

April 11, 1939.

L. McCULLOCH

2,154,276

FILLING COMPOUND FOR AND METHOD OF INSULATING CONDUCTORS

Filed Feb. 17, 1938



WITNESSES:

Wm. B. Sellers.  
James M. Ely

INVENTOR

Leon McCulloch.

BY

Gran W. Savage  
ATTORNEY

## UNITED STATES PATENT OFFICE

2,154,276

FILLING COMPOUND FOR AND METHOD OF  
INSULATING CONDUCTORS

Leon McCulloch, Pittsburgh, Pa., assignor to Westinghouse Electric & Manufacturing Company, East Pittsburgh, Pa., a corporation of Pennsylvania

Application February 17, 1938, Serial No. 191,037

## 8 Claims. (Cl. 106—15)

This invention relates to filling compounds for bushings and to the insulating of the conductors from the weather casings of bushings.

In manufacturing bushings, the space between the conductor element and the weather casing is filled with an insulating material, such as oil or the like. In many applications, and in particular the bushings employed in conjunction with power transformers, oil is not altogether satisfactory as a filling material because the high operating temperature which is encountered makes it quite difficult to maintain a tight seal of the oil-filled bushing.

The gum compounds sometimes employed heretofore as the filling material are not entirely satisfactory in that they have one or more defects. Some of the gum compounds employed have too high a dielectric power factor or have the defect that they are of so low density compared with water that water may sink therein and be entrapped. Another defect of certain of these gum compounds is that they have a tendency to become so hard and brittle at temperatures below 0° F. as to contract and form voids and cracks with the result that moisture can enter and corona may occur.

An object of this invention is the provision of a filling compound suitable for use in bushings.

Another object of this invention is the provision of a filling compound for use in bushings which is heavier than water and soft at low temperatures.

A further object of this invention is to protect electrical apparatus provided with a bushing in which a conductor element is disposed in spaced relation to a weather casing by interposing a suitable filling compound between the conductor and the casing to increase the dielectric strength of the path from the conductor to the casing.

Another object of this invention is to provide for insulating a casing from a conductor disposed in spaced relation therein.

Other objects of this invention will become apparent from the following description when taken in conjunction with the accompanying drawing, the single figure of which is shown in elevation and partly in section, illustrates a transformer provided with a bushing that is protected in accordance with the teachings of this invention.

Referring to the drawing, this invention is illustrated with reference to a transformer 10 having a core 12 and coils 14 immersed in an insulating and cooling medium 16 within a suitable casing 18. The casing 18 carries suitable lead-in bushings 20, which, in this instance, are illustrated

as being of the condenser type, the conductors 22 or condenser elements of which are spaced from the weather casing 24 of porcelain or other suitable dielectric material and connected to the coil assembly by suitable leads 26. As illustrated, 5 a filling compound 28 is employed in the bushing to fill the space between the conductor elements and the weather casing of the bushing.

In preparing the filling compound, it is desirable to employ a base material which may be 10 melted and become fluid enough for pouring into the space between the conductor elements and the weather casing. It is also desirable that the base material be resilient and rubbery at ordinary temperatures and have the property of being 15 more or less elastic at lower temperatures.

Asphalt, and particularly petroleum asphalt which is substantially free from mineral impurities, has these desirable properties and is preferred to be employed as the base material. A 20 preferred petroleum asphalt employed as the base material is one which may be purchased on the open market and has the properties of having a Ball and Ring melting point of 115° C., a penetration of 15 seconds at 25° C., a pouring temperature of 175° C., a specific gravity of 1.02 at 20° C., 25 and is less than 0.6% insoluble in benzol.

Since the petroleum asphalt has a density less than that of water, in order to increase the density to a value substantially above that of 30 water, a chlorinated hydrocarbon is added to the asphalt. The chlorinated hydrocarbon employed for this purpose is one of those known in the open market as the aroclors which are derived from diphenyl and its derivatives and which has 35 a chlorine content of between 55% and 70% and a preferred chlorine content of between 60% and 65%. The preferred aroclor is selected from that group of aroclors which are non-crystalline, 40 glassy, resin-like solids at room temperature and are soluble in oil in all proportions.

The non-crystalline aroclors are the chlorinated high boiling derivatives of diphenyl fractionated, the fractionating boiling range being between 270° C. and 400° C. as prepared by the 45 well known synthetic manufacture of diphenyl by passing the vapors of benzene through molten lead and subsequently fractionation of the product. These aroclors have extremely high chemical stability, being resistant to oxidation and the 50 effects of moisture at moderately elevated temperatures without liberation of acid, and are of very low volatility. Further, they have no appreciable swelling or softening action upon varnishes, and will, therefore, not effect the var- 55

nished paper-wound condenser elements when employed in the filling compound for condenser bushings.

In order that the filling compound may have the desired softness at low temperatures, a light oil is employed in conjunction with the asphalt and the aroclor. In order to prevent softening of the varnish on the condenser elements of a condenser bushing, the oil employed must be of a non-aromatic nature. A preferred oil is the refined petroleum oil known as transformer oil such as may be purchased on the open market having excellent electrical properties, low viscosity, low freezing point, and is stable, inert and non-volatile at ordinary temperatures.

In preparing the compound, it is desirable to mix the asphalt, aroclor and oil in such proportions that it will have a density greater than that of water. A compound having a density of 1.05 at 20° C. is found to be satisfactory, since it floats water and still does not contain so large a proportion of the aroclor as to prohibitively increase the cost of the final compound. The following table lists a number of the representative compounds having the required properties and which are satisfactory for use as a filling compound in the bushings.

#### Composition

| Serial No. | Aroclor | Asphalt | Oil |
|------------|---------|---------|-----|
| 183        | 17      | 60      | 23  |
| 253        | 17      | 58      | 25  |
| 254        | 18      | 56      | 26  |
| 255        | 18      | 54      | 28  |
| 35 185     | 20      | 40      | 40  |

These compounds have a specific gravity of about 1.05 at 20° C. and a "pull away" temperature of between -40° F. and -85° F.

The "pull away" temperature of the filling compound is a measure of the hardness of the compound at low temperatures, and may be determined by placing a quantity of the compound in a large glass tube which is then stoppered and immersed in an alcohol bath. When immersed in the alcohol bath, the temperature of the bath is lowered in steps of 10° F. by employing solid carbon dioxide and holding the bath at each particular temperature for a period of time of about thirty minutes. When the temperature of the bath is sufficiently lowered, the compound within the glass tube hardens and contracts enough to separate suddenly from the walls of the glass tube emitting a loud cracking sound. The temperature at which this occurs is called the "pull-away" temperature. Where the "pull-away" temperature is -40° F. or lower, the compound is satisfactory as a filling compound for bushings.

The compounds prepared as hereinbefore described are quite viscous as may be readily determined by following with X-rays the rise of large air bubbles through the compounds in two-inch glass tubes inclined at an angle of 22° and kept at a temperature of about 25° C. In testing the compound identified hereinbefore as No. 183, it is found that the bubble of air travels 7 inches in 48 hours, while in compound No. 253, the bubble of air travels 8 inches in a corresponding period.

In these compounds, the non-crystalline aroclors stabilize the solution of the asphalt in the mineral oil and render the compound stable at the surface even after long exposure to water.

The resistance of the compound toward water is

because of the high solvent power of the aroclor for the oil and the asphalt.

The compound described hereinbefore is sufficiently dielectric that, when employed as a filling compound in the bushing structure, it increases the dielectric strength of the path from the conductor elements within the bushing to the casing and metal supporting flange of the bushing. Further, since the compound is heavier than water and resistant to moisture penetration as well as having the characteristic of being a substantially viscous gum down to temperatures of the order of -40° F. or lower, the compound will function to exclude water or moisture from the elements under substantially all conditions which may be met in service. These compounds, because of their uniform quality and relatively good chemical stability and the ease with which they may be melted and poured or run into the space between a conductor element and a casing, may easily be interposed between the conductor element and the casing of extremely slender bushing assemblies.

Although this invention has been described with reference to a particular compound, it is, of course, not to be limited thereto except insofar as is necessitated by the prior art and the scope of the appended claims.

I claim as my invention:

1. A filling compound for bushings comprising a petroleum asphalt, a chlorinated hydrocarbon having the characteristic of being a non-crystalline, glassy, resin-like solid at room temperature, and a petroleum oil.

2. A filling compound for bushings comprising a petroleum asphalt, a chlorinated hydrocarbon selected from the group of aroclors having a chlorine content of between 55 and 70%, and a petroleum oil.

3. A filling compound for bushings comprising from 40 to 60% of petroleum asphalt, from 17 to 29% of aroclor having a chlorine content of between 55 and 70%, and from 23 to 40% of petroleum oil.

4. A filling compound for bushings comprising about 58% of petroleum asphalt, about 17% of aroclor having a chlorine content of between 55 and 70%, and about 25% of petroleum oil.

5. A filling compound for bushings comprising from 54 to 60% of petroleum asphalt, from about 17 to 18% of a chlorinated hydrocarbon selected from the group of aroclors having a chlorine content of between 60 and 65%, and from about 23 to 28% of petroleum oil.

6. The method of protecting electrical apparatus provided with a bushing in which a conductor element is disposed in spaced relation to a weather casing comprising interposing between the conductor and casing a dielectric filling compound which comprises a petroleum asphalt, a chlorinated hydrocarbon selected from the group of aroclors having a chlorine content of between 55 and 70% and petroleum oil to increase the dielectric strength of the path from the conductor element to the casing and exclude moisture from the element.

7. The method of protecting electrical apparatus provided with a bushing in which a conductor element is disposed in spaced relation to a weather casing comprising interposing between the conductor and casing a dielectric filling compound which comprises from 40 to 60% of petroleum asphalt, from 17 to 20% of a chlorinated hydrocarbon selected from the group of aroclors having a chlorine content of between 55 and 70%.

and from about 23 to 40% of petroleum oil, which compound increases the dielectric strength of the path from the conductor element to the casing and excludes moisture from the element.

5 8. The method of insulating a conductor from a casing which comprises interposing a dielectric filling compound between the conductor and cas-

ing, the dielectric filling compound comprising from 54 to 60% of petroleum asphalt, from 17 to 18% of a chlorinated hydrocarbon selected from the group of aroclors having a chlorine content of between about 55 and 70% and from 23 to 28% of petroleum oil. <sup>5</sup>

LEON McCULLOCH.